



above-mentioned compound in which all four R radicals are hydroxypropyl radicals and the radical R' is ethylene, the preferred amount to use in the cadmium cyanide plating bath is about 0.5 gram per liter, although some effect is produced with as little as 0.1 gram per liter, while 1 gram per liter can be used without ill effects.

Similar amounts of each of the other above-mentioned compounds may likewise be used in cadmium cyanide plating baths with some noticeable effect in each instance.

While my novel cadmium cyanide plating bath addition agents are effective in any operable cadmium cyanide plating solution, I prefer to use a bath having the general formula,

|                      | Grams per liter |
|----------------------|-----------------|
| Sodium cyanide, NaCN | 120             |
| Cadmium oxide, CdO   | 26              |

My novel cadmium cyanide plating bath addition agents have numerous advantages over other such materials now being used commercially. They are not only brighteners, but also anti-pit agents, so that no secondary materials are needed to prevent pitting of deposits. Another advantage is that my novel brighteners are definite chemical compounds whose composition can be controlled and duplicated, in distinction to those brighteners which contain organic matter of unknown composition. Still another advantage is that my novel brighteners act as sequestering agents for the deleterious metallic impurities, such as copper for example, that commonly contaminate cadmium cyanide plating baths in commercial operation, thus preventing the harmful effects of such impurities. Still another advantage is that my novel addition agents act effectively as brighteners on the anodes as well as on the cathodes, so as to keep the anode surfaces bright and clean. They act to promote uniform anode corrosion and prevent selective attack at the crystal boundaries, which results in fine metallic particles being dispersed in the bath, which migrate to the cathode, thereby producing rough deposits.

Still another advantage is the high degree of stability of my novel cadmium plating addition agents in the alkaline cadmium cyanide plating bath under operating conditions, which makes for economy, since only the brightener lost by bath dragout needs to be replaced.

While my novel cadmium cyanide plating bath addition agents are effective when used alone in cadmium cyanide plating baths, it is expedient for some purposes to combine them with other materials that act synergistically to produce certain desirable results under some conditions. For example, they may be used in combination with certain colloidal materials to improve the brightness of deposit and coverage in the low current density areas on irregularly shaped objects, particularly in barrel plating solutions. As examples of colloidal materials suitable for use with my novel cadmium cyanide plating bath addition agents, I may cite gelatin, peptone, and hydroxy ethyl cellulose, the last named being preferred. These materials are added to the plating bath to produce concentrations of from about 0.1 to 1 gram per liter, but in general not greater than the concentration of my novel addition agent in the bath at the time.

In order to broaden the bright plating current density range, particularly in the higher ranges, I have found it expedient to add a soluble nickel or cobalt salt as taught in U. S. Patent, 1,681,509. Any bath soluble compound of nickel may be used to produce a bath concentration of approximately 0.02 to 0.2 gram of nickel per liter, but in general the nickel concentration should not be greater than about one-fifth the concentration of my novel addition agent in the bath at the time.

It is apparent from the foregoing that under certain conditions it will be advantageous to use mixtures of one or more of my novel brighteners with a colloidal material. As an example of such a mixture that I have found to be effective is a mixture of N,N,N<sup>1</sup>,N<sup>1</sup> tetrakis

(2-hydroxy ethyl) ethylene diamine one part and hydroxy ethyl cellulose one part, the mixture being added to the bath to produce a concentration of about one gram of the mixture per liter of plating bath. Under other conditions, it will be advantageous to use mixtures of one or more of my novel brighteners with a bath soluble nickel compound. A convenient compound for this purpose is crystalline nickel sulfate, NiSO<sub>4</sub>·7H<sub>2</sub>O. One such mixture that I have found to be effective is N,N,N,N<sup>1</sup> tetrakis (2-hydroxy butyl) ethylene diamine, one part, and NiSO<sub>4</sub>·7H<sub>2</sub>O, one part, the mixture being added to the bath to produce a concentration of about one gram of the mixture per liter of plating bath.

I have found that mixture addition agents can be compounded so as to produce superior results over the wide range of operating conditions encountered with commercial cadmium cyanide plating baths. Such mixtures are made by mixing one or more of my novel addition agents with a colloidal material and a bath soluble nickel compound. For convenience, such addition agents are best compounded in the form of a solution portions of which can be added to a cadmium cyanide plating bath. As an example of one such solution that I found to produce particularly good results, I cite the following formulation:

|                                                                                 | Grams per liter |
|---------------------------------------------------------------------------------|-----------------|
| N,N,N <sup>1</sup> ,N <sup>1</sup> tetrakis (2-hydroxy propyl) ethylene diamine | 20              |
| Hydroxy ethyl cellulose                                                         | 10              |
| NiSO <sub>4</sub> ·7H <sub>2</sub> O                                            | 10              |

This mixed addition agent solution is then added to a cadmium cyanide plating bath in the proportion of about 18 cc. of addition agent solution per liter of plating bath, or about 250 fluid ounces of mixed addition agent solution per 100 gallons of plating bath.

#### Example 1

A general formula for such mixed addition agent formulations coming within the scope of my invention would be:

|                                                                                | Parts |
|--------------------------------------------------------------------------------|-------|
| N,N,N <sup>1</sup> ,N <sup>1</sup> - tetrakis (hydroxy alkyl) ethylene diamine | 20    |
| Hydroxy ethyl cellulose                                                        | 10    |
| NiSO <sub>4</sub> ·7H <sub>2</sub> O                                           | 20    |
| Water                                                                          | 950   |

Other compounds which come within the scope of my invention and have been found to give satisfactory results are illustrated in Examples Nos. 2 and 3:

#### Example 2

|                                                    | Parts |
|----------------------------------------------------|-------|
| Monohydroxyethyl trihydroxypropyl ethylene diamine | 18    |
| Peptone                                            | 12    |
| NiSO <sub>4</sub> ·7H <sub>2</sub> O               | 16    |
| Water                                              | 954   |

#### Example 3

|                                                 |     |
|-------------------------------------------------|-----|
| Dihydroxyethyl dihydroxypropyl ethylene diamine | 16  |
| Gelatin                                         | 13  |
| NiSO <sub>4</sub> ·7H <sub>2</sub> O            | 14  |
| Water                                           | 957 |

This application is a continuation-in-part of my co-pending application Serial No. 481,969, filed January 14, 1955, now abandoned.

While the invention has been described as embodied in concrete form and as operating in a specific manner in accordance with the provisions of the patent statutes, it should be understood that the invention is not limited thereto, since various modifications will suggest themselves to those skilled in the art without departing from the spirit of the invention, the scope of which is set forth in the annexed claims.

I claim:

1. A cadmium cyanide plating bath composition containing a totally hydroxyalkylated ethylene diamine having the formula



in which each R is an alkyl radical containing from 2 to 4 carbon atoms, in a concentration of about 0.1 to about 1 gram per liter.

2. A cadmium cyanide plating bath composition containing a totally hydroxyalkylated ethylene diamine having the formula



where each R is an alkyl radical containing from 2 to 4 carbon atoms, in a concentration from about 0.1 to about 1 gram per liter and a colloid selected from the group consisting of gelatin, peptone, and hydroxyethyl cellulose in a concentration of about 0.1 to about 1 gram per liter.

3. A cadmium cyanide plating bath composition containing a totally hydroxyalkylated ethylene diamine having the formula



where each R is an alkyl radical containing from 2 to 4 carbon atoms, in a concentration of about 0.1 to 1 gram per liter and nickel in bath soluble form in a concentration of about 0.02 to 0.2 gram per liter.

4. A cadmium cyanide plating bath composition containing a totally hydroxyalkylated ethylene diamine having the formula



where each R is an alkyl radical containing from 2 to 4 carbon atoms, and a colloid selected from the group consisting of gelatin, peptone, and hydroxyethyl cellulose, each being in concentration of about 0.1 to 1 gram per liter, and nickel in bath soluble form in a concentration of about 0.02 to 0.2 gram per liter.

5. A cadmium cyanide plating bath composition containing N,N,N<sup>1</sup>,N<sup>1</sup>-tetrakis (2-hydroxy propyl) ethylene diamine in a concentration of about 0.1 to 1 gram per liter.

6. A cadmium cyanide plating bath composition containing N,N,N<sup>1</sup>,N<sup>1</sup>-tetrakis (2-hydroxy ethyl) ethylene diamine and a colloid selected from the group consisting of gelatin, peptone, and hydroxyethyl cellulose, each in concentration of about 0.1 to 1 gram per liter.

7. A cadmium cyanide plating bath composition containing N,N,N<sup>1</sup>,N<sup>1</sup>-tetrakis (2-hydroxy butyl) ethylene diamine in a concentration of about 0.1 to 1 gram per liter and nickel in bath soluble form in concentration of about 0.02 to 0.2 gram per liter.

8. A cadmium cyanide plating bath composition containing N,N,N<sup>1</sup>,N<sup>1</sup>-tetrakis (2-hydroxy propyl) ethylene diamine and hydroxyethyl cellulose, each in a concentration of about 0.1 to 1 gram per liter and nickel in bath soluble form in a concentration of about 0.02 to 0.2 gram per liter.

9. A composition of matter for use in cadmium cyanide electroplating baths containing totally hydroxyalkylated ethylene diamine in which all the alkyl substituents contain from 2 to 4 carbon atoms, a colloid selected from the group consisting of gelatin, peptone, and hydroxyethyl cellulose, and nickel in bath soluble form in proportions

to each other effective when added to a cadmium cyanide plating bath to produce the bath composition of claim 4.

10. A liquid addition agent for use in cadmium cyanide electroplating baths containing in aqueous solution, N,N,N<sup>1</sup>,N<sup>1</sup>-tetrakis (2-hydroxy propyl) ethylene diamine one part, hydroxyethyl cellulose in amount equal to from about one-fifth part to one part, and nickel in the form of water soluble salt equivalent to nickel from about one-twenty-fifth part to one-fifth part.

11. A liquid addition agent for use in cadmium cyanide electroplating baths containing in aqueous solution, N,N,N<sup>1</sup>,N<sup>1</sup>-tetrakis (2-hydroxy propyl) ethylene diamine one part and hydroxyethyl cellulose one part, and nickel in the form of a water soluble compound in proportion of approximately one-fifth part of nickel.

12. A cadmium cyanide plating bath addition composition containing substantially equal parts of N,N,N<sup>1</sup>,N<sup>1</sup>-tetrakis (hydroxy propyl) ethylene diamine, a colloid selected from the group consisting of gelatin, peptone, and hydroxyethyl cellulose, and nickel in bath soluble form.

13. A cadmium cyanide plating bath addition composition containing about one part of N,N,N<sup>1</sup>,N<sup>1</sup>-tetrakis (2-hydroxy propyl) ethylene diamine and between about one-fifth part and about one part of hydroxyethyl cellulose.

14. A cadmium cyanide plating bath addition composition containing about one part of N,N,N<sup>1</sup>,N<sup>1</sup>-tetrakis (2-hydroxy propyl) ethylene diamine and between about one twenty-fifth part and about one part of nickel in the form of a water soluble salt.

15. A cadmium cyanide plating bath composition containing a totally hydroxyalkylated alkylene diamine having the formula



in which each R and R' is an alkyl radical containing from 2 to 4 carbon atoms, in a concentration of about 0.1 to about 1 gram per liter.

16. A cadmium cyanide plating bath composition containing a totally hydroxyalkylated alkylene diamine having the formula



in which each R is an alkyl radical containing from 2 to 4 carbon atoms and R' is a propyl radical, in a concentration of about 0.1 to about 1 gram per liter.

17. A cadmium cyanide plating bath composition containing a totally hydroxyalkylated alkylene diamine having the formula



in which each R is an alkyl radical containing from 2 to 4 carbon atoms and R' is a butyl radical, in a concentration of about 0.1 to about 1 gram per liter.

18. A cadmium cyanide plating bath composition containing a totally hydroxyalkylated alkylene diamine having the formula



where each R and R' is an alkyl radical containing from 2 to 4 carbon atoms, and a colloid selected from the group consisting of gelatin, peptone, and hydroxyethyl cellulose, each being in concentration of about 0.1 to 1 gram per liter, and nickel in bath soluble form in a concentration of about 0.02 to 0.2 gram per liter.

19. A composition of matter for use in cadmium cyanide electroplating baths containing a totally hydroxy-alkylated alkylene diamine having the formula



in which each R and R' is an alkyl radical containing from 2 to 4 carbon atoms, a colloid selected from the group consisting of gelatin, peptone, and hydroxyethyl cellulose, and nickel in bath soluble form in proportions to each other effective when added to a cadmium cyanide plating bath to produce the bath composition of claim 18.

20. A composition of matter for use in cadmium cyanide electroplating baths containing a totally hydroxy-alkylated alkylene diamine having the formula



in which each R is an alkyl radical containing from 2 to 4 carbon atoms and R' is a propyl radical, a colloid selected from the group consisting of gelatin, peptone and hydroxyethyl cellulose, each being in concentration of about 0.1 to 1 gram per liter, and nickel in bath soluble

form in a concentration of about 0.02 to 0.2 gram per liter.

21. A composition of matter for use in cadmium cyanide electroplating baths containing a totally hydroxy-alkylated alkylene diamine having the formula



in which each R is an alkyl radical containing from 2 to 4 carbon atoms and R' is a butyl radical, a colloid selected from the group consisting of gelatin, peptone and hydroxyethyl cellulose, each being in concentration of about 0.1 gram to 1 gram per liter, and nickel in bath soluble form in a concentration of about 0.02 to 0.2 gram per liter.

References Cited in the file of this patent

FOREIGN PATENTS

731,102 Germany Feb. 3, 1943

OTHER REFERENCES

"Sequestrene," Alrose Chemical Co., Providence, R. I., July 25, 1952, page 28.